

P. BUNET.

PROCESS FOR THE MANUFACTURE OF ALUMINIUM NITRID.

APPLICATION FILED MAY 9, 1913.

1,145,747.

Patented July 6, 1915.

2 SHEETS—SHEET 1.



Witnesses:  
Hallen Abbe  
W. E. Keis

Inventor  
Paul Bunet  
By his Attorneys  
Howe and Townsend

1,145,747.

P. BUNET,  
PROCESS FOR THE MANUFACTURE OF ALUMINIUM NITRID,  
APPLICATION FILED MAY 9, 1913.

Patented July 6, 1915.

2 SHEETS—SHEET 2.

Fig. 3.



Fig. 4.



Witnesses:

Walter Abbr  
W. E. Kerr

Inventor  
Paul Bunet  
By his Attorney  
Howson and Howson

# UNITED STATES PATENT OFFICE.

PAUL BUNET, OF WHITNEY, NORTH CAROLINA, ASSIGNOR TO SOCIÉTÉ GÉNÉRALE DES NITRURES, OF PARIS, FRANCE.

## PROCESS FOR THE MANUFACTURE OF ALUMINIUM NITRID.

1,145,747.

Specification of Letters Patent.

Patented July 6, 1915.

Application filed May 9, 1913. Serial No. 766,461.

To all whom it may concern:

Be it known that I, PAUL BUNET, of Whitney, Stanly county, North Carolina, and a citizen of the Republic of France, have invented certain new and useful Improvements in Processes for the Manufacture of Aluminium Nitrid, of which the following is a full, clear, and exact description.

This invention relates to a process for the manufacture of aluminium nitrid by the method which consists in heating in presence of nitrogen or of gases containing the latter, a mixture of alumina or aluminous substances and carbon in an electrical resistance furnace in which the material under treatment itself serves as the heating resistance.

The invention consists in effecting the advance in the continuous electrical furnace of the mixture of the above substances containing an excess of carbon or other conductive substances in sufficient quantity to insure the passage of current in spite of the reactionary losses of carbon, necessary to the transformation of the alumina into aluminium nitrid.

The operation may take place in an electrical furnace of any kind, in which the material under treatment itself serves as the heating resistance. It is, however, carried out preferably in one or other of the types of furnace hereafter described.

The first type of furnace is arranged in such a way that the thickness of the layer of material goes on increasing in proportion as the latter advances through the furnace. In this way the sectional area increases in the parts of the furnace where the mixture becomes poor in carbon in consequence of the reaction, and there is, therefore, always at every cross-section of the furnace a sufficient quantity of conductive material to insure the regular passage of the current.

The second type of furnace is so arranged that at intervals along its length there are connections or electrodes for conveying the current, which are connected alternately to the two poles of the generator or supply. In this way the furnace is divided into a number of elements or sections through which the material under treatment passes successively; the length of each section can be selected in accordance with the state of conductivity of the material treated therein.

These two types of furnace can evidently be combined.

The accompanying drawing shows by way of examples various forms of construction of furnaces for carrying out the process.

Figure 1 is a longitudinal section, illustrating an inclined revolving electric furnace, according to my invention; Fig. 2 is a vertical section of a stationary form of furnace; Figs. 3 and 4 are diagrammatic sections of two modified forms of revolving electric furnaces.

Fig. 1 shows a revolving furnace, which is slightly inclined so as to allow the substances introduced into the furnace to advance therethrough in a continuous manner, after the general manner described in the Serpek Patent, No. 1,030,929, July 2, 1912. The gaseous current containing nitrogen circulates, as usual, in the contrary direction to the materials. The electric current is led to two annular conductors A and B of which the lower one B projects inside the furnace so as to form a diaphragm and to retain the material C traveling through the furnace.

As explained above, in proportion as the material advances through the furnace and the transformation into nitrid becomes more complete, the thickness of the layer is increased, in this way allowing of maintaining at every cross section the quantity of carbon sufficient to insure the regular passage of the current in spite of the losses resulting from the reaction. Matters can, therefore, be so arranged that the resistance and consequently the evolution of heat are approximately constant throughout the length of the furnace.

In order to heat up the furnace and to facilitate the passage of the current at the start, the operation may be commenced by passing carbon alone through the furnace; the mixture to be treated is then gradually added. There may be arranged in the furnace at certain intervals conductive rings D fitted in the refractory lining, E, and projecting or not. In this way there are formed in the furnace zones of less resistance which facilitate the passage of the current. This arrangement allows the furnace to be made of any length, greater in proportion to the size of the projections of the conductive rings D.

Fig. 2 of the drawings shows a stationary furnace based upon the same principle; the furnace is vertical and the current is led

to the two electrodes  $A^1$  and  $B^1$ . The material poured upon the side of the electrode  $A^1$  falls upon the lateral walls of the furnace forming a sloping bank, the sectional area of which increases toward the lower electrode  $B^1$ . The electrode  $A^1$  is insulated on its underside on an insulating support  $A^2$  in order that the current shall pass with certainty through the mixture  $C^1$  under treatment. The electrode  $A^1$  and its support  $A^2$  are movable and can be raised or lowered; in this way the furnace is regulated by increasing or decreasing the separation of the electrodes and the areas for the passage of the mixture. Openings  $F$ , closed by plugs  $F^1$ , are formed at the bottom of the furnace at various points in the periphery to allow the material to be withdrawn.

20 Fig. 3 is a longitudinal section of a furnace of the second type, in which an intermediate electrode or terminal  $B^2$  is arranged between the extreme electrodes  $A^3$ ,  $A^4$ , all these electrodes being formed as conductive rings or annuli.

Fig. 4 is a longitudinal section of a similar furnace, having two intermediate electrodes; in this case some of the conductive rings forming terminals have been arranged 30 to project internally of the furnace so as to afford walls or diaphragms according to the principle of the first type of furnace above described.

In the arrangement of Fig. 4, the conductive rings  $A^3$ ,  $A^4$  are connected to one of the poles of the electrical generator while the alternate rings  $B^3$ ,  $B^4$  are connected to the other pole.

40 In these two figures,  $E$  still indicates the refractory lining of the furnace and  $C$  the material in course of its advance therethrough. The current of nitrogen circulates in the opposite direction as usual.

The use of intermediate electrodes and 45 the possibility of selecting their separation as desired, form a practical method which allows latitude for regulating in accordance with the requirement of manufacture one or more of the following factors which are 50 all of importance in the management of revolving electrical furnaces, viz:—voltage, resistance, current intensity, length and inclination of the furnace, proportion of the conductive material added to the mass in reaction, total expenditure of energy and 55 of heat and division of the matter along the various elementary sections of the furnace.

In particular, by reducing the length of 60 the path traveled by the material between two successive electrodes, the resistance is diminished. It becomes possible, therefore, to reduce the quantity of conducting material added to the materials in reaction in order to insure the passage of the current; this allows of diminishing the expenditure

of energy devoted to the heating of these conductive materials and to obtain at the end of the operation a product which is not surcharged with inert material and is, therefore, richer in nitrid. Instead of reducing 70 the proportion of conductive matter added, the length of the furnace may be increased without reaching a resistance deleterious to the satisfactory carrying out of the operation. In this way there is obtained a result 75 analogous to that which is produced by the conductive rings  $D$ , which are not connected to the poles of the generator in the furnace shown in Fig. 1. Again, by bringing closer together two consecutive 80 electrodes, the heat may be concentrated in a given zone as desired, for example in the final zone which is the poorest in carbon and in which the current has most difficulty in passing.

Another peculiarity of the type of furnace, which presents an important practical advantage, lies in the fact that it realizes automatically the regulation of the intensity of the current, and, therefore, of the 85 quantity of heat which passes through the different elementary sections of the furnace. Indeed, if for any reason the intensity of the current increased abnormally at one of the sections of the furnace, to the detriment 90 of the others, there would be produced at that point a larger quantity of heat; this would increase the reaction of the carbon and alumina. There would result an elimination 95 of carbon in the state of carbon monoxid and the reacting mixture would become less conductive; this would cause a reduction in the intensity of the current in this section and so reestablish the general equilibrium.

100 As has been said before, it is advantageous to combine the use of intermediate electrodes with the system of furnace-diaphragms as shown in Fig. 1; such an arrangement is illustrated in Fig. 4. In this 105 way it becomes possible to combine the useful effects of the methods of regulation of the two systems, according to different requirements. In particular, it becomes possible to vary as desired in each elementary 110 section of the furnace, the thickness of the layer of material under treatment, and the extent which it occupies between two consecutive electrodes.

115 As stated above, the material delivered to the furnace may be a mixture of alumina and carbon with an excess of the latter over or above the quantity necessary to the reaction. By way of example, it may be stated that there may be introduced into the mixture a quantity of carbon double that which is necessary to the reaction. A part or the whole of this excess of carbon may, however, equally well be replaced by one or more substances which are good electrical 120

conductors, the metals for example. Among these substances, it is of advantage to select those which possess at the same time the property of actifying the reaction of formation of nitrid. One may, for example, use iron, copper, nickel, manganese or their ores or again alloys of these metals, such as ferro-nickel, ferro-silicon, ferro-manganese, etc. The use of iron or of certain of its alloys has the further special advantage of allowing it to be separated magnetically from the aluminium nitrid at the end of the operation.

Since iron oxid is already found in greater or less proportions in certain aluminium ores, (in particular the ferruginous bauxites, for example), it will be sufficient in case of the use of these ores to complete by additions the quantity of iron required to obtain the desired conductivity of the mass under treatment.

The material introduced into the furnace (whatever be its composition and whatever be the type of furnace employed) may be in the pulverulent state or in the form of agglomerates; it may again be in the form of agglomerates containing only the alumina or aluminous material and the carbon necessary to the reaction, while the carbon or other conductive material intended to insure the desired conductivity is added separately. In case the conductive material added consists wholly or in part of carbon, the atmospheric air may be used directly as the gas of the reaction; the excess of carbon contained in the material may then serve at the end of the operation and beyond the electrical zone to deprive this air of its oxygen.

In carrying out my above described process of manufacturing aluminium nitrid, I do not restrict myself to the use of the construction of furnace described. That construction will form the subject of a divisional application.

45 I claim as my invention:

1. As an improvement in the process for the manufacture of aluminium nitrid by heating in presence of nitrogen a mixture of aluminous material and carbon, the process consisting in causing to advance in a continuous electrical furnace the mixture of reactionary materials with an addition of conductive materials which at the same time actify the reaction.

55 2. As an improvement in the process for the manufacture of aluminium nitrid by heating in presence of nitrogen a mixture of aluminous material and carbon, the process consisting in causing to advance in a continuous electrical furnace the mixture of reactionary materials with an addition of conductive material, which actifies the reaction and is also separable magnetically at the end of the operation.

65 3. As an improvement in the process for

the manufacture of aluminium nitrid by heating in presence of nitrogen a mixture of aluminous material and carbon, the process consisting in causing to advance in a continuous electrical furnace the mixture of reactionary materials with an addition of conductive material sufficient to insure in all cases the passage of the current, notwithstanding the losses due to the reactions, the material treated being in the form of agglomerates, substantially as described.

70 4. As an improvement in the process for the manufacture of aluminium nitrid by heating in presence of nitrogen a mixture of aluminous material and carbon, the process consisting in causing to advance in a continuous electrical furnace the mixture of reactionary materials with an addition of conductive material sufficient to insure in all cases the passage of the current, notwithstanding the losses due to the reactions, the layer of material treated increasing toward the outlet end of the furnace, substantially as described.

75 5. As an improvement in the process for the manufacture of aluminium nitrid by heating in presence of nitrogen a mixture of aluminous material and carbon, the process consisting in causing to advance in a continuous electrical furnace the mixture of reactionary materials with an addition or excess of carbon, and supplying air to the furnace at the delivery end, thereby providing gas containing nitrogen by the freeing of the atmospheric air of its oxygen by the excess of carbon still contained in the materials at the delivery end.

80 6. The herein described method of heating materials by means of electrical energy, which consists in establishing in a rotary furnace having a highly insulating lining a charge of high electrical conductivity relative to the lining, passing a heating current through the charge, whereby the current is confined practically to the charge and heats the same by the resistance thereof, and supplying to one end of the furnace material to be heated and withdrawing material from the other end while rotating the furnace.

85 7. The herein described method of heating materials by means of electrical energy, which consists in establishing in a rotary furnace having a highly insulating lining a charge composed of commingled conducting and non-conducting materials, and passing a heating current through said charge while rotating the furnace.

90 8. The herein described method of heating granular non-conducting materials by means of electrical energy, which consists in establishing in a rotary furnace having a highly insulating lining a charge containing non-conducting material in granular form and conductive material in the form of relatively large masses of lumps, passing a heat-

ing current through the charge while rotating the furnace, and supplying granular non-conducting material to one end of the furnace and withdrawing such material 5 from the other end while retaining inside the furnace the said lumps or masses of conducting material.

9. The herein described method of heating non-conducting aluminiferous material in 10 the presence of gaseous nitrogen for the production of aluminum nitrid, which consists in establishing in a rotary furnace having a highly insulating and refractory lining a

charge containing such non-conducting aluminiferous material and refractory conducting material, and passing a heating current through the charge while rotating the furnace and passing a current of nitrogen through the furnace. 15

In testimony whereof I have signed my name to this specification, in the presence of two subscribing witnesses.

PAUL BUNET.

Witnesses:

WALTER ABBE,  
HUBERT HOWEN.